

Patented Mar. 19, 1929.

1,706,294

# UNITED STATES PATENT OFFICE.

ISADORE M. JACOBSON, OF CHICAGO, ILLINOIS, AND STARR TRUSCOTT, OF BIRMINGHAM, OHIO.

## AIRCRAFT COVERING.

No Drawing.

Application filed April 11, 1925. Serial No. 22,348.

This invention relates to improvements in flexible gas retaining fabrics for aircraft and more particularly to the gas retaining fabric used in the gas cells of aircraft of the 5 Zeppelin type.

One of the objects of the present invention is to provide an impermeable flexible membrane or covering of the above general character which may be inexpensively manufactured and fabricated into gas retaining bags or cells.

A further object is to provide a fabric of the above general character adapted to eliminate the use of goldbeaters' skins heretofore 10 considered essential.

Other objects will be in part obvious and in part hereinafter pointed out.

It is our belief that cellulose, except in the form of its esters and ethers, has not previously been dispersed in any of the solvents 20 capable of dispersing rubber. From the results of experiments we are convinced that films prepared from such dispersions of cellulose and rubber have very high resistance 25 to the passage of gases. These films may be applied to a base cloth or fabric or produced independently and applied to cloth or fabric by means of cement. There are doubtless other uses to which this material 30 may be put.

In order to obtain cellulose in the form in which it may be dispersed in organic solvents viscose, or other aqueous dispersion of cellulose derivative, and latex are thoroughly mixed. If desired, accelerators, activators, antioxidants, and other materials which have been found to give desirable properties to rubber compounds may be incorporated in the mixture. They may be 35 added in the beginning, or may be milled into the coagulated mixture at a later stage or may be added to the dispersion of the mixture in the organic solvent.

When the entire mixture has become homogeneous the mixture is poured, or forced 45 through an orifice, or passed in any other manner into a bath capable of coagulating the viscose-latex mixture. The product is allowed to remain in this bath until completely coagulated. It is then washed thoroughly with water in order to remove all 50 water soluble material contained in it. This product is then drained and dried preferably by passing a current of air over or through it at normal temperatures. When

dried it is milled a sufficient length of time so that it may readily be dispersed in the medium desired. The following examples will illustrate the method.

Two thousand gms. of viscose, prepared 60 from 150 gms. of cellulose, namely, cotton linters, is mixed thoroughly with 375 gms. of rubber latex, containing 40% of non-volatile material. The mixture obtained is poured into a bath containing a 10% solution of acetic acid, in a fine stream such that a heavy thread is formed upon coagulation. The thickness of this thread should be not over 2 to 3 mm. in order to facilitate washing and drying. The coagulated mass is 65 allowed to remain in the coagulating bath for a period of three hours. After this time it is drained and washed thoroughly in running cold water until the washings no longer show an acid reaction. The product is then drained and air dried, whereupon 70 its color changes from white to translucent yellow or brown. This dried material is milled for a period of fifteen minutes.

Two hundred and fifty gms. of this milled 75 product are suspended in 750 gms. of benzene and allowed to stand over night in a stoppered vessel, at room temperature. The following morning, a large proportion of the material will be found to be dispersed. 80 The residue on the bottom of the vessel may be dispersed by vigorous agitation. After standing for weeks, only a comparatively small amount of the incompletely dispersed material separates.

The viscose must not have aged excessively at the time of use. Swollen fibrous particles will separate from the mixture of old viscose and latex. The length of time which viscose may be kept without excessive 90 deterioration depends upon the temperature at which it is kept, decomposition occurring more rapidly at higher temperatures. We have found it possible, however, to use viscose which has been stored in a glass vessel 95 kept in an ice chest for as long as 15 to 20 days. The viscose-latex mixture should be kept at a temperature not exceeding 20° C.

We do not confine ourselves in this patent to the proportions referred to above, to the use of acetic acid as a coagulating medium, to the method of drying, time of milling, or to the use of benzene as a dispersing medium for the product obtained.

It will thus be seen that the present in- 110

vention provides a simple and practical fabric for use on aircraft adapted to accomplish, among others, all of the objects and advantages herein set forth.

5. What we claim as our invention is:
1. A fabric treated with a compound consisting of a mixture of regenerated cellulose and rubber redispersed in organic solvents.
  2. A method of rendering a fabric flexi-

ble and impermeable to gases consisting in 10  
coating the fabric with sizing and applying  
thereto a layer of a mixture of regenerated  
cellulose and rubber redispersed in organic  
solvents.

Signed at Washington, District of Colum- 15  
bia, this ninth day of January, 1925.

ISADORE M. JACOBSON.  
STARR TRUSCOTT.